

No. 687,531.

Patented Nov. 26, 1901.

C. W. JEFFERSON.  
INSULATING MATERIAL.

(Application filed Feb. 7, 1901.)

(No Model.)



**WITNESSES:**

John O. Gumpel.  
Edwin Seeger.

**INVENTOR**

INVENTOR  
Charles W. Jefferson

BY  
Kenyon & Kenyon  
ATTORNEYS

# UNITED STATES PATENT OFFICE.

CHARLES W. JEFFERSON, OF SCHENECTADY, NEW YORK, ASSIGNOR TO THE MICA INSULATOR COMPANY, A CORPORATION OF NEW JERSEY.

## INSULATING MATERIAL.

SPECIFICATION forming part of Letters Patent No. 687,531, dated November 26, 1901.

Application filed February 7, 1901. Serial No. 46,305. (No model.)

*To all whom it may concern:*

Be it known that I, CHARLES W. JEFFERSON, a subject of the Queen of Great Britain, and a resident of Schenectady, in the county of Schenectady and State of New York, have invented certain new and useful Improvements in Insulating Material, of which the following is a specification.

My invention relates to compound insulating materials; and it has for its object the manufacture of such a material that will not only be thoroughly flexible, pliable, and non-brittle, but that will also be able to resist a very high electrical voltage and to withstand a very great degree of heat.

Electrical insulators have been made in the shape of plates or sheets and of some comminuted or pulverized non-combustible insulating material mixed with a hardening cement. One of the disadvantages of this kind of insulator is that it is not pliable and that it is brittle and also that it has not the required efficiency as to insulation and durability, and the plates or sheets so made being brittle and non-pliable are more apt to chip and break when being manipulated or cut into smaller pieces for insulation. In order to remedy these defects and to give the sheet more durability and flexibility, sheets of fabric have sometimes been introduced into the combined insulating sheet or plate; but the disadvantage of the use of such fabric is that it is readily carbonized, and as soon as this happens the efficiency of the insulator is impaired. Sheets of insulating material have also been made from layers of scales of mica cemented by a varnish and then the sheet so formed dried by steam and then subjected to intense pressure, so that the varnish between the mica scales and between the layers will be expelled, leaving only sufficient of the varnish to cause the mica scales to adhere together. The plate or sheet so formed is then subjected to intense pressure, so that the different layers of mica scales are formed into a compact sheet in a hard state. A sheet of insulation constructed as above described makes a very good insulator; but as the sheet itself is virtually composed of a solid mass of mica it is somewhat brittle and not as pliable

as is sometimes desired. Also with such a construction of insulating-sheet it is liable to crack, especially when cut into smaller pieces or trimmed. By my invention a very simple, inexpensive, pliable, non-brittle, and highly-efficient insulating material can be constructed.

My invention consists of the insulated material herein described.

In the accompanying drawings, Figure 1 illustrates in perspective a sheet of insulating material showing one embodiment of my invention, said sheet being broken away at different parts to clearly show the construction. Fig. 2 is a fragmentary view, enlarged, in plan and showing how the different scales of mica may be laid and are united. Fig. 3 is a fragmentary cross-section, greatly magnified, of portion of the insulating-sheet illustrated by Fig. 1. Fig. 4 is a similar view to Fig. 1, but showing a slightly-modified form of insulated sheet. Fig. 5 illustrates the mechanism which may be used in one stage of the process of making the insulating-sheet.

Similar numbers represent like parts in all the figures.

1 represents the pliable substance forming the body of my improved insulating-sheet and also arranged in alternate layers.

2 represents layers formed of mica scales 3, said layers 2 being united by the substance 1 and the spaces between the scales 3 and the layers 2 being filled in with said substance.

4 represents the flexible composition cover or coating of the insulated sheet.

5, Fig. 4, represents sheets of tissue-paper or other flexible porous material saturated with an insulating compound and forming part of the sheet and interposed between the outer layer and the coating or cover 4.

6 represents a body-plate of a table 7, which plate may be heated or cooled by means of a pipe 8 passing under said plate.

9 is a light roller to be used in pressing down the different layers of the sheet during the process of manufacture and for expelling gas from the same.

The method I prefer to use in the manufacture of my improved insulating material

is as follows: A layer of insulating material in a fluid or semifluid state is first applied to a base-plate 6, said plate having previously been coated with soapstone or some similar material, so that after said layer has become hardened, or partly so, it may be readily scaled from the plate. The material which I prefer to use is an oxidized oil, and preferably oxidized linseed-oil, as such oxidized oil forms in itself a very good insulator and is quite pliable when oxidized or dried. In order to produce the best results, I take linseed-oil which has first been oxidized and then dissolve it with benzine or some similar solvent. Then I prefer to add to this dissolved oxidized oil a very small proportion of some gum, as copal-gum. This gives the oil a little more of an adhesive quality and a little more body. After the liquid above described is applied in a layer 1 to the base-plate 6, as above stated, a layer 2 of mica scales 3 is laid on the layer 1 of said liquid, preferably overlapping each other, then another layer 1 of the liquid is applied over the layer of mica scales, and this process is continued until the sheet is of the desired thickness, said sheet being made of alternate layers 1 of the insulating liquid or semiliquid and of mica scales 3. When the sheet is of the desired thickness, the plate 6 is then heated preferably, by steam from a pipe 8. The highly-volatile quality of the benzine or other solvent will have caused it to evaporate to some extent even before the plate is heated, thus turning the oil or other liquid into a gum, uniting the different mica scales and layers of the same. The heat from the plate will cause still more evaporation of the solvent and tend to dry the oxidized oil. During said evaporation and drying, while the sheet is still upon the plate, a light pressure is applied to the sheet by means of a roller 9 or other device, such pressure being sufficient to smooth and level the layers of oxidized oil and mica scales and to expel the gas from the sheet; but such pressure must not be sufficient to squeeze out the oil or other binding compound, as such oil, which is now transformed into a gum, is to constitute the main portion 1 of the insulating-sheet. The sheet is then put in an oven for a short time and dried. It is then taken out of the oven and coated by dipping or otherwise in the dissolved oxidized oil or other liquid, thus forming a coating or cover 4 to the sheet, and then hung up in the oven—say with a temperature of about 100° Fahrenheit—for about two hours, with a heat gradually increasing to about 400° Fahrenheit. The temperature of the oven is then gradually reduced for about two hours to about the degree of heat that the plate first became subjected to, which might be in the neighborhood of 100° Fahrenheit. The oxidized sheet (see Fig. 1) is now complete, and it is of a very pliable character, with the oxidized and baked oil 1 forming the main part or body of the sheet filling in all the spaces

between the mica scales 3 and between the layers of the same and uniting said scales and layers, so that the completed sheet is formed in one solid mass.

Although I prefer to bake the sheet, as above stated, to procure the best results, such sheet may be dried in any appropriate manner.

The "scales" of mica that I prefer to use in the manufacture of my new insulating material are such elementary or primary scales as are understood in mineralogy as being the thinnest sheets or single layers of mica that can be practically obtained by the continued process of cleavage or splitting. The object of forming the insulating material of such thin elementary scales is to prevent all liability of the different pieces of mica splitting, which the scales might do if they were thicker, and thus cause a splitting or separation of different parts of the insulating material, there being no oxidized oil or other adhesive substance between the separated layers of a double or multiple layered scale of mica. Even a partial separation of different parts of an insulator would leave a space for air and moisture, and thus impair the efficiency of the insulator. By reason of the use of a pliable adhesive insulating substance the finely-divided mica scales can be united in a solid mass with said substance, so that the resultant product is a sheet or body of very flexible and pliable insulating material that can be bent, doubled up, and twisted in any manner desired to suit the various forms and conditions for which insulators are used. If the adhesive substance that binds the mica scales together were not of a flexible and pliable nature, the completed insulating product could not be bent and twisted without liability of breaking.

The different layers of oxidized oil or other liquid may be applied with a brush or in any other appropriate manner, and the scales of the different layers should preferably overlap those of the other layers, so that the resistance offered to an electrical current in an insulator so formed would be transverse to the surfaces of the mica scales, there being always, besides the oxidized insulating compound, a scale of mica to resist the force of the electrical current. Still better results may be attained by a second coating of the plate with the dissolved oxidized oil, and it should then preferably be hung up in the oven in a reverse position to that in which it was suspended before. When this second baking is contemplated, it will not be necessary to keep the sheet in the oven quite as long the first time, (or it may be otherwise dried,) as the second baking will effect the desired result of thoroughly oxidizing and hardening the oil or body of the sheet and of uniting said body with the mica scales in a solid mass.

The insulating-sheet made by my improved method has been found to be most efficient

as an insulator, and it will withstand a very high degree of heat and also a very high electrical voltage, higher than that of any compound insulating material so far known to me.

5 The insulating-sheet may be slightly modified in form by applying a sheet 5 of thin porous material, (see Fig. 4,) such as tissue-paper, to one or both of the outside layers 1 of the insulating compound previous to the drying and pressing stages of the process, and then dipping such covered or coated sheet in the said compound, and then baking in the oven, as above described. When this form of sheet is made, very small scales of mica 15 may be used, and it will not be necessary to use as many layers of said scales as when the tissue-paper or other fabric is omitted, as the layer or layers 5 of flexible material will form a durable binder for the entire sheet. The 20 oxidized composition will thoroughly impregnate the tissue-paper or other fabric and render it virtually non-carbonizable. The efficiency of said sheet as an insulator is equal to that in which the coating of flexible fabric 25 is omitted.

By practical experience I find that the insulators made in accordance with my invention will resist at least fifteen hundred volts to one-thousandth of an inch in thickness of 30 said insulators.

What I claim as new, and desire to secure by Letters Patent, is—

1. The improved insulating material, consisting of layers of a pliable, adhesive, binding substance, and layers of the thinnest or primary mica scales, the said layers united to form a solid pliable mass.

2. The improved insulating material, consisting of layers of a pliable, adhesive, insulating substance, and layers of the thinnest or primary mica scales overlapping each other, the said layers united to form a solid pliable mass.

3. The improved insulating material, consisting of layers of a pliable, adhesive, insulating substance, and layers of the thinnest or primary mica scales, the said layers united to form a solid pliable mass, and said mass having a coating of said substance.

5 4. The improved insulating material, consisting of layers of a pliable, adhesive, insulating substance, and layers of the thinnest or primary mica scales overlapping each other, the said layers united to form a solid pliable mass, and said mass having a coating of said substance.

5 5. The improved insulating material, consisting of layers of a pliable, adhesive, insulating substance, and layers of the thinnest or primary mica scales, the said layers united to form a solid pliable mass, said mass being covered with a layer of thin, porous, flexible material, and said mass and layer having a coating of said substance.

65 6. The improved insulating material, consisting of layers of a pliable, adhesive, oxi-

dized binding substance, and layers of the thinnest or primary mica scales, the said layers united to form a solid pliable mass.

7. The improved insulating material, consisting of layers of a pliable, adhesive, oxidized insulating substance, and layers of the thinnest or primary mica scales overlapping each other, the said layers united to form a solid pliable mass. 70

8. The improved insulating material, consisting of layers of oxidized oil and of mica scales.

9. The improved insulating material, consisting of layers of oxidized oil and of single- 80 layer or primary mica scales.

10. The improved insulating material, consisting of layers of oxidized oil and of single-layer or primary mica scales, said oxidized oil forming a substantial part of the body of 85 the insulating material and uniting said scales to form a solid mass.

11. The improved insulating material, consisting of layers of oxidized oil and of irregularly-shaped mica scales. 90

12. The improved insulating material, consisting of layers of oxidized oil and of overlapping mica scales.

13. The improved insulating material, consisting of insulating oxidized oil, and layers 95 of mica scales, said oxidized oil forming a substantial part of the body of the insulating material, and uniting said scales to form a solid mass.

14. The improved insulating material, consisting of insulating oxidized oil, and layers of mica scales overlapping each other, said oxidized oil forming a substantial part of the body of the insulating material, and uniting said scales to form a solid mass. 100

15. The improved insulating material, consisting of oxidized linseed-oil, and layers of mica scales, said oxidized oil forming a substantial part of the body of the insulating material, and uniting said scales to form a solid 105 mass with the same.

16. The improved insulating material, consisting of oxidized linseed-oil, and layers of mica scales overlapping each other, said oxidized oil forming a substantial part of the body of 115 the insulating material, and uniting said scales to form a solid mass.

17. The improved insulating material, consisting of insulating oxidized oil, and mica scales overlapping each other, said oxidized oil 120 forming a substantial part of the body of the insulating material, and uniting said scales to form a solid mass, and said mass having a coating of said oxidized oil.

18. The improved insulating material, consisting of oxidized linseed-oil, and mica scales overlapping each other, said oxidized oil forming a substantial part of the body of the insulating material, and uniting said scales to form a solid mass, and said mass having a 125 coating of said oxidized oil. 130

19. The improved insulating material, con-

sisting of layers of oxidized oil and of irregularly-shaped overlapping mica scales.

20. The improved insulating material, consisting of layers of oxidized oil and of irregularly-shaped single-layer or primary mica scales.

21. The improved insulating material, consisting of layers of oxidized oil and of overlapping single-layer or primary mica scales.

22. The improved insulating material, consisting of layers of oxidized oil and of irregularly-shaped overlapping single-layer or primary mica scales.

23. The improved insulating material, consisting of layers of oxidized oil and of irregularly-shaped single-layer or primary mica scales, said oxidized oil forming a substantial part of the body of the insulating material and uniting said scales to form a solid mass.

24. The improved insulating material, consisting of layers of oxidized oil and of overlapping single-layer or primary mica scales, said oxidized oil forming a substantial part of the body of the insulating material and uniting said scales to form a solid mass.

25. The improved insulating material, consisting of layers of oxidized oil and of irregularly-shaped overlapping single-layer or primary mica scales, said oxidized oil forming a substantial part of the body of the insulating material and uniting said scales to form a solid mass.

26. The improved insulating material, consisting of a pliable, dissolvable and adhesive insulating substance, and layers of mica scales, said substance forming a substantial part of the body of the insulating material, and uniting said scales to form a solid mass, and said mass having a coating of said substance.

27. The improved insulating material, consisting of a pliable, dissolvable and adhesive oxidized insulating substance, and mica scales

overlapping each other, said substance forming a substantial part of the body of the insulating material, and uniting said scales to 45 form a solid mass, said mass being covered with a layer of thin porous flexible material, and said mass and layer having a coating of said substance.

28. The improved insulating material, consisting of a pliable, dissolvable and adhesive oxidized insulating substance, and mica scales overlapping each other, said substance forming a substantial part of the body of the insulating material, and uniting said scales to 55 form a solid mass, said mass being covered with a layer of tissue-paper, and said mass and layer having a coating of said substance.

29. The improved insulating material, consisting of a pliable, dissolvable and adhesive 60 oxidized insulating substance, and layers of mica scales, said substance forming a substantial part of the body of the insulating material, and uniting said scales to form a solid mass, said mass being covered with a layer of 65 thin porous flexible material, and said mass and layer having a coating of said substance.

30. The improved insulating material, consisting of a pliable, dissolvable and adhesive oxidized insulating substance, and layers of 70 mica scales overlapping each other, said substance forming a substantial part of the body of the insulating material, and uniting said scales and layers to form a solid mass, said mass being covered with a layer of thin porous flexible material, and said mass and layer having a coating of said substance.

In testimony whereof I have signed my name to this specification in the presence of two subscribing witnesses.

CHARLES W. JEFFERSON.

Witnesses:

ALLAN H. JACKSON,  
HOMER STRONG.